



US006432223B1

(12) **United States Patent**  
Bartholomeusz et al.

(10) **Patent No.:** US 6,432,223 B1  
(45) **Date of Patent:** Aug. 13, 2002

(54) **MAGNETIC DATA-STORAGE TARGETS AND METHOD FOR PREPARATION**

5,411,604 A \* 5/1995 Inokuti ..... 148/112  
5,500,057 A 3/1996 Inoue et al.

(75) Inventors: **Michael Bartholomeusz, Michael Tsai,**  
both of Chandler, AZ (US)

## FOREIGN PATENT DOCUMENTS

JP 60-2624 \* 8/1985

(73) Assignee: **Heraeus Inc.**, Chandler, AZ (US)

## OTHER PUBLICATIONS

(\*) Notice: Subject to any disclaimer, the term of this  
patent is extended or adjusted under 35  
U.S.C. 154(b) by 0 days.

A Dictionary of Metallurgy, MacDonald & Evans, Ltd.  
London, 1958, p. 269.\*

(21) Appl. No.: **09/546,015**

"Improved Magnetic Behaviour of Cobalt-Based-Alloy  
Sputter-Target Material", by Weigert et al., Materials Science and Engineering, A139 (1991) 359-363.

(22) Filed: **Apr. 10, 2000**

"Magnetic Properties and Microstructure of Co-Cr Bulk  
Alloys", by Chan et al., Journal of Magnetism and Magnetic  
Materials, 79 (1989) 95-108.

## Related U.S. Application Data

Encyclopedia of Chemical Technology, 3<sup>rd</sup> Ed., vol. 15,  
John Wiley & Sons, New York, pp. 325-345.

(62) Division of application No. 08/946,360, filed on Oct. 7,  
1997, now Pat. No. 6,123,783.

\* cited by examiner

(60) Provisional application No. 60/038,031, filed on Feb. 6,  
1997.

Primary Examiner—John Sheehan

(51) **Int. Cl.<sup>7</sup>** ..... **H01F 1/147**

(74) Attorney, Agent, or Firm—McDermott, Will & Emery

(52) **U.S. Cl.** ..... **148/120**

## ABSTRACT

(58) **Field of Search** ..... 148/110, 111,  
148/112, 120, 121

A method for making a magnetic data storage target includes  
warm-rolling a magnetic alloy sheet at a temperature of less  
than about 1200° F., optimally followed by annealing. The  
method results in increased pass-through-flux (PTF) and  
improved performance in magnetron sputtering applica-  
tions.

(56) **References Cited**

## U.S. PATENT DOCUMENTS

4,702,780 A \* 10/1987 Inokuti et al. ..... 148/111  
5,334,267 A 8/1994 Taniguchi et al.

**21 Claims, 26 Drawing Sheets**



Relationship between PTF and maximum material permeability



Depiction of bar magnet and axial Hall probe contact  
PTF measurement technique.

$$PTF = \frac{H_{app}}{H_{trans}}$$

FIG. 1



Grain Size Distribution

**FIG. 2**  
(PRIOR ART)



VSM B-H loop for Ni target fabricated using standard techniques known in the prior art

FIG. 3  
(PRIOR ART)



XRD spectrum for Ni target fabricated using standard techniques known in the prior art

FIG. 4 (PRIOR ART)



FIG. 5



XRD spectrum for Ni target fabricated using the straight warm-rolled practice

FIG. 6

Functional inverse relation between PTF and  $U_{max}$ 

FIG. 7



XRD spectrum for Co target fabricated using standard techniques known in the prior art

FIG. 8 (PRIOR ART)



XRD spectrum of Co target fabricated using the  
straight warm-rolled practice

FIG. 9



FIG. 10



FIG. 11(a)

XRD spectrum for Co-10Cr-4Ta targets  
fabricated using process (1)



XRD spectrum for Co-10Cr-4Ta targets  
fabricated using process (2)

FIG. 11(b)



XRD spectrum for Co-10Cr-4Ta targets  
fabricated using process (3)

FIG. 11(c)



XRD spectrum for Co-12Cr-4Ta-10Ni targets  
fabricated using process (1)

FIG. 12(a)



XRD spectrum for Co-12Cr-4Ta-10Ni targets  
fabricated using process (2)

FIG. 12(b)



XRD spectrum for Co-12Cr-4Ta-10Ni targets  
fabricated using process (3)

FIG. 12(c)



VSM data for Co-10Cr-4Ta targets  
fabricated using process (1)

FIG. 13(a)



FIG. 13(b)



VSM data for Co-10Cr-4Ta targets  
fabricated using process (3)

FIG. 13(c)



VSM data for Co-12Cr-4Ta-10Ni targets  
fabricated using process (1)

FIG. 14(a)



VSM data for Co-12Cr-4Ta-10Ni targets  
fabricated using process (2)

FIG. 14(b)



VSM data for Co-12Cr-4Ta-10Ni targets  
fabricated using process (3)

FIG. 14(c)



FIG. 15



FIG. 16



Effect of uniaxial warm-rolling on grain aspect ratio

FIG. 17



Relationship between PTF and maximum material permeability

FIG. 18

## MAGNETIC DATA-STORAGE TARGETS AND METHOD FOR PREPARATION

### CROSS REFERENCE TO RELATED APPLICATION

This application is a Divisional of application Ser. No. 08/946,360 filed Oct. 7, 1997, now U.S. Pat. No. 6,123,783. This application claims priority of Provisional Application Serial No. 60/038,031, filed on Feb. 6, 1997.

### FIELD OF THE INVENTION

The present invention relates to the fabrication of magnetic target materials and more specifically to methods of producing magnetic target materials with low permeabilities and high pass-through-flux (PTF) characteristics. In particular, the invention relates to methods for increasing PTF by metallurgically inducing a reduction in target material permeability which promotes enhanced sputtering efficiency, better target material utilization and improved sputtered film thickness uniformity.

### BACKGROUND OF THE INVENTION

Magnetron sputtering involves the arrangement of permanent or electromagnets behind a target material (cathode), and applying a magnetic field to the target. The applied magnetic field transmits through the target and focuses a discharge plasma onto the front of the target. The target front surface is atomized with subsequent deposition of the target atoms on top of an evolving thin film device positioned adjacent to the target.

Magnetron sputtering of magnetic target materials is very prevalent in the electronics industry, particularly in the fabrication of semiconductor and data storage devices. Due to the soft magnetic nature of magnetic target alloys, there is considerable shunting of the applied magnetic field in the bulk of the target. This in turn results in reduced target utilization due to focussing of the transmitted magnetic field in the erosion groove formed as a result of the shunting. This focussing effect is exacerbated with increasing material permeability (which corresponds to decreasing material PTF).

It is well known that reducing target material permeability promotes a less severe erosion profile which enhances target material utilization and subsequently contributes to a reduction in material cost. The presence of severe target erosion profiles also promotes a point source sputtering phenomena which can result in less than optimum deposited film thickness uniformity. Therefore, decreasing target material permeability has the added benefit of increasing deposited film thickness uniformity.

The PTF of a magnetic target is defined as the ratio of transmitted magnetic field to applied magnetic field. A PTF value of 100% is indicative of a non-magnetic material where none of the applied field is shunted through the bulk of the target. The PTF of magnetic target materials is typically specified in the range of 0 to 100%, with the majority of commercially produced materials exhibiting values between 10 to 95%.

There are several different techniques for measuring product PTF. One technique involves placing a 4.4 (+/-0.4) kilogauss bar magnet in contact on one side of the target material and monitoring the transmitted field using a axial Hall probe in contact on the other side of the target material. The maximum value of the magnetic field transmitted through the bulk of the target divided by the applied field

strength in the absence of the target between the magnet and probe (maintained at the same distance apart as when the target was between them) is defined as the PTF. PTF can be expressed as either a fraction or a percent.

Another technique for measuring PTF involves using a horseshoe magnet and a transverse Hall probe. The PTF values measured using different magnet and probe arrangements are found to exhibit good linear correlation for the values of magnet field strength typically utilized in the industry. The PTF measurement techniques are constructed to realistically approximate the applied magnetic flux occurring in an actual magnetron sputtering machine. Therefore, PTF measurements have direct applicability to a target material's performance during magnetron sputtering. FIG. 1 depicts the bar magnet and axial Hall probe contact PTF measurement set-up utilized for the measurements discussed hereafter.

Magnetic material PTF and permeability are not mutually exclusive. Rather, there is a very strong inverse correlation between PTF and maximum permeability of magnetic materials. Values of material magnetic permeability can be very precisely determined by using vibrating-sample-magnetometer (VSM) techniques in accordance with ASTM Standard A 894-89. Descriptions of sample geometry and calculation of the appropriate demagnetization factors for permeability determination are well known in the art. See, for example, Bozarth, *Ferromagnetism*, p. 846.

Magnetic target PTF is a strong function of both target chemistry and the thermomechanical techniques utilized during target fabrication. For alloys that do not possess inherently high PTF as a result of their stoichiometry (PTF<85%), it is possible to increase product PTF by various thermomechanical manipulations during product fabrication.

Typical fabrication of Ni, Co and Co-alloy targets involves casting, hot-rolling and either heat treatment or cold-rolling or a combination of heat treatment followed by cold-rolling. It is known, for example, that heat treating and cold-rolling of magnetic target materials can increase product PTF. Heat treatment of Co—Cr—Ta—(Pt) alloys below 2200° F. has been shown to increase the PTF by promoting matrix crystallographic phase transformation from FCC (face centered cubic) to HCP (hexagonal close packed). The driving force for this martensitic transformation is provided by the interfacial strain associated with the precipitation of Co—Ta semi-coherent precipitates during heat treatment. Chan et al., *Magnetism and Magnetic Materials*, vol. 79, pp 95-108 (1989), suggests that the greater mobility of domain walls in the HCP phase compared with the FCC phase in Co—Cr base alloys contributes to the increase in target PTF with microstructural phase transformation from FCC to HCP.

It is suggested in Weigert et al., *Mat. Sci. and Eng.*, A 139, pp 359-363 (1991), that cold-rolling of (62 to 80 atomic %)Co-(18 to 30 atomic %)Ni-(0 to 8 atomic %)Cr alloys immediately after the hot-rolling process results in an increase in product PTF. This suggests that the increase in PTF is a result of the cold-deformation induced [0001] basal hexagonal texture ([0001] hexagonal directions aligned perpendicular to the target surface). A similar result is disclosed in Uchida et al., U.S. Pat. No. 5,468,305 for Co-(0.1 to 40 atomic %)Ni-(0.1 to 40 atomic %)Pt-(4 to 25 atomic %)Cr alloys cold-rolled by not more than a 10% total reduction after the hot-rolling process. Uchida et al. claim that the cold-deformation induces internal strain in the alloy which reduces magnetic permeability. As mentioned earlier, a

reduction in magnetic permeability corresponds to an increase in product PTF.

In summary, the prior art teaches cold-rolling as a means of increasing product PTF by either enhancing the basal texture component of the HCP phase or increasing the overall alloy internal strain density. It is possible that both the texture and strain mechanisms promote an overall increase alloy PTF.

Three issues are specifically not addressed in the prior art: (1) The utilization of warm-rolling practices to enhance product PTF, (2) The very pronounced effect of directionality during hot and cold-rolling on product PTF and (3) the further enhancement of target material PTF by employing post warm-rolling heat treatment practices.

Current data storage technology utilizes a myriad of multi-component multi-phasic alloys that tend to be very hard and brittle. Adverse effects associated with cold-rolling of these alloys include the following: (1) severe deformation results in a high risk of plate cracking, warping and chipping; (2) large residual stresses result in significant difficulties during final product machining; (3) a substantial amount of wear and damage to the rolling mills typically used to process these materials; and (4) due to the severity of the cold-rolling process, the overall reduction is commonly not enough to guarantee uniform strain and texture gradients throughout the thickness of the part.

The presence of microstructural gradients in the part can be deleterious to product consistency during final sputtering application which involves the successive atomic removal of material from the target surface. The combination of these factors results in high product cost and less than optimum performance consistency.

Thus, despite the advantages of using cold-rolling for increasing PTF, there remains a need in the art for an improved process which further increases pass-through-flux and eliminates the problems associated with cold-rolling.

#### SUMMARY OF THE INVENTION

The present invention meets the above need. It is according to an aspect of the invention to provide a method for increasing the pass-through-flux of a magnetic target beyond that achievable using cold-rolling.

It is another aspect of the invention to provide a method, as above, which increases the pronounced directionality effect on PTF observed during hot and cold-rolling.

It is yet another aspect of the invention to provide a method, as above, which decreases the risk of plate (target sheet) cracking, warping and chipping compared to cold-rolled targets.

It is still another aspect of the invention to provide a method, as above, which decreases residual stresses in the target compared to cold-rolled targets.

It is yet another aspect of the invention to provide a method, as above, which provides more uniform strain and texture gradients throughout the thickness of the target.

These aspects and others discussed hereafter, are achieved in the broadest sense by a process for warm-rolling a magnetic metal or metal alloy with at least one component thereof being a magnetic metal.

In a particular embodiment, the metal-containing article formed by the process is a magnetic target useful in magnetron sputtering.

The aspects of the invention are also achieved by a method for forming a magnetic sheet material by hot-rolling a magnetic metal or a metal alloy including a magnetic

metal, thereby forming a sheet, cold water quenching the sheet and then warm-rolling the quenched sheet at a temperature of less than about 1200° F. to achieve a reduction in sheet thickness of at least about 15%, thereby forming a magnetic sheet material.

The aspects of the invention are also achieved by a magnetic target material comprising a sheet formed by warm-rolling a magnetic metal or a metal alloy including a magnetic metal, having a pass-through-flux of at least about 30% and an average grain length-to-width aspect ratio of greater than about 1.1 in the rolling direction.

#### BRIEF DESCRIPTION OF THE DRAWINGS

For a fuller understanding of the invention, the following detailed description should be read in conjunction with the drawings, wherein:

FIG. 1 shows a schematic representation of a bar magnet and an axial Hall probe, and a schematic representation of a bar magnet and an axial Hall probe with a target inserted;

FIG. 2 is a histogram illustrating grain-size distribution of an Ni target;

FIG. 3 is a VSM B-H loop for an Ni target fabricated according to the prior art;

FIG. 4 is an x-ray diffraction (XRD) spectrum for an Ni target fabricated according to the prior art;

FIG. 5 is a histogram illustrating grain size distribution of an Ni target;

FIG. 6 is an XRD spectrum for an Ni target fabricated using a straight warm-rolled technique of the invention;

FIG. 7 is a graph illustrating the functional inverse relationship between PTF and Umax;

FIG. 8 is an XRD spectrum of a Co target fabricated according to the prior art;

FIG. 9 is an XRD spectrum for a Co target fabricated using the straight warm-rolling technique of the present invention;

FIG. 10 is an XRD spectrum for a cobalt target fabricated using the post straight warm-roll annealing technique of the present invention;

FIGS. 11(a)–(c) are XRD spectra for a Co-10Cr-4Ta target fabricated according to Example 3;

FIGS. 12 (a)–(c) are XRD spectra for a Co-10Cr-4Ta-10Ni target fabricated according to Example 3;

FIGS. 13(a)–(c) are graphs of VSM data for Co-10Cr-4Ta targets fabricated according to Example 3;

FIGS. 14(a)–(c) are graphs of VSM data for a Co-12Cr-4Ta-10Ni target fabricated according to Example 3;

FIG. 15 is a graph of the effect of uni-axial warm-rolling on PTF;

FIG. 16 is a graph of the effect of uni-axial warm-rolling on texture;

FIG. 17 is a graph of the effect of uni-axial warm-rolling on grain aspect ratio;

FIG. 18 is a graph of the relationship between PTF and maximum material permeability.

#### DETAILED DESCRIPTION OF THE PREFERRED DESCRIPTION

While the following description sets forth the method of the invention in the context of forming magnetic targets for magnetron sputtering techniques, it is emphasized that the scope of the invention broadly encompasses other environments for the magnetic metal and metal alloys formed by the method.

In general, the method of the invention may be used to modify known prior art techniques for forming magnetic articles in which pass-through-flux is an important feature. Thus, known techniques for forming magnetic articles by rolling can be modified to incorporate warm-rolling as discussed hereinafter.

The invention contemplates the use of magnetic metals in either relatively pure form or in the form of metal alloys. Pure metals include Ni and Co. The preferred metals and metal alloys are encompassed by the following formula



wherein the values of a-d are atomic weight% basis and wherein a is 0-100%; b is 0-40%; c is 0-8%; and d is the remainder. In addition, from 0 to 30% (atomic), based on 100% of the above alloy, of one or more of the following secondary elements can be added: Pt, B, Si, Zr, Fe, W, Mo, V, Nb, Hf, Ti and Sm. The secondary elements may be used to enhance deposited film characteristics such as reduced signal to noise ratio and enhanced coercivity.

Prior art techniques for forming magnetic articles, such as targets for magnetron sputtering, have included the steps of melting the metal or metal alloy, casting it to form an ingot, and then hot-rolling the ingot at a temperature of from 2200° F. to 1400° F. This produces a total reduction of sheet thickness of between 30 and 65% and functions to reduce porosity in the ingot. After hot-rolling, the ingot is quenched in cold water, followed by cold-rolling at near ambient temperature and/or heat treating at a temperature between about 800° F. and about 1600° F.

In the present invention, a warm-rolling step is provided either after, or as a replacement for, cold-rolling and heat treating.

The warm-rolling step provides for a thickness reduction of at least about 3% and as high as about 85% or even higher. Desirably the reduction is from about 15% to about 75% and preferably from about 20% to about 70%. In a highly preferred embodiment the warm-rolling step produces a thickness reduction of from about 25% to about 40%.

Depending on the desired thickness reduction, the warm-rolling can be performed in a single pass or in multiple passes. Each pass through the rollers may produce a thickness reduction of from about 2% to about 50%. In a preferred embodiment, the rollers are set to provide a thickness reduction of from about 2% to about 25%. In a less preferred, but still advantageous embodiment, the rollers are set to provide a thickness reduction of from about 25% to about 50% per pass.

If multiple passes are performed, the directional orientation of any one pass in relation to the other pass or passes can have an effect on the physical properties of the final product. Multiple pass rolling (both warm and cold) may be performed in one of several, for example, clock rolling, cross rolling and straight rolling. In clock rolling the sheet is turned clockwise (or counterclockwise) a specified number of degrees after each rolling step. For example, in a 3 pass rolling process, the sheet may be turned 1200 after each rolling step. In cross rolling, the sheet is rolled alternatively at 90° angles from the previous rolling step. In straight rolling, all rolling steps are performed in the same direction.

In a highly preferred embodiment, multi-pass warm-rolling is performed in the same direction (straight warm-rolling) at a reduction of between about 2% and 25% per pass, for a total reduction of from about 20% to about 70%.

Warm-rolling is performed at a temperature lower than the hot-rolling step, that is, below about 1400° F. Generally warm-rolling is performed at a temperature of less than

about 1350° F., desirably less than about 1300° F. and preferably less than about 1200° F., for examples at between about 600° F. and about 1100° F. All temperatures refer to the temperature of the sheet at the time of rolling.

In another preferred embodiment, the sheet is annealed before warm-rolling, after warm-rolling, or both. The annealing step is believed to reduce strain in the microstructure caused by the warm-rolling. Generally the annealing step is carried out at a temperature of from about 600° F. to about 1600° F. (sheet temperature) for a period of from about 1 to about 6 hours.

It has been found that, as an alternative to cold-rolling, warm-rolling of magnetic materials can promote equivalent increases in product PTF as obtained with cold-rolling, and is accompanied by the following advantages: significantly reduced plate cracking during processing; lower non-uniform residual stresses in the finished part (target); diminished rolling mill wear and tear during processing; and more uniform microstructural gradients in the finished part due to the greater rolling reductions achievable. It has empirically been found that for many alloys, product PTF can be significantly enhanced (or Umax concomitantly reduced) by warm-rolling below 1200° F. for a total reduction of between 3% to 65% (total reduction is defined as  $dt/t \times 100\%$ , where  $t$  is the starting thickness prior to warm-rolling and  $dt$  is the total reduction in thickness after warm-rolling).

In the data-storage industry, maximizing target PTF has become an important method for optimizing product utilization and stability of the sputtering process. In this regard, it has been discovered that, quite unexpectedly, unidirectional warm-rolling, as opposed to cross, clock, symmetric or bi-directional warm-rolling, further increases PTF. Thus, in a highly preferred embodiment, the warm-rolling is performed in a straight line (straight warm-rolling). Straight warm-rolling has been found to yield the most favorable product microstructural texture required to promote maximum PTF.

For the various magnetic target alloys, straight warm-rolling results in final product PTF between 40% to 95% for final product thickness between 0.050" to 0.500".

The microstructural manifestation of straight warm-rolling is an average product grain length-to-width aspect ratio greater than about 1.4 in the rolling direction and preferably greater than about 1.6. It has also been discovered that the application of post warm-roll thermal treatments to promote a further increase in product PTF over and above that of simply warm-rolling.

The following Examples illustrate the invention.

In the following Examples 1, 2, and 3, warm rolling is conducted at a temperature of about 1100° F. with the sheet being reheated if the sheet temperature falls below about 500° F.

#### EXAMPLE 1

##### Fabrication of Ni Target Product

Two ingots of 99.995 pure Ni were vacuum induction melted. Ingot #1 was fabricated using practices available in the prior art: The ingot was hot-rolled at between 2200° F. and 1400° F. for a total reduction of 65% to heal any as-cast porosity in the ingot. After hot-rolling, the ingot was cold water quenched and cold clock-rolled for a total reduction of another 65% to inject enough deformation induced nucleation sites for subsequent recrystallization. Clock-rolling is a process of rotating the plate in a clockwise, or counter clockwise fashion, by some incremental amount (30 to 90 degrees) after every pass in the rolling mill in preparation for

the next pass. After cold clock-rolling the plate was heat treated in the temperature range of about 1000° F. for 1 hour to promote microstructural recrystallization. Finally, the plate was machined into a final target product of thickness 0.118" (+/-0.005") The resulting product exhibited the following microstructural and magnetic properties:

|                                           |                                |
|-------------------------------------------|--------------------------------|
| Grain size =                              | 40 (+/-17) micrometers surface |
|                                           | 97 (+/-40) micrometers center  |
| Grain size gradient (surface-to-center) = | 57 micrometers                 |
| PTF =                                     | 15%                            |

FIG. 2 depicts the grain size distribution of the target fabricated from ingot #1. The average grain sizes at the target surface and center were calculated in accordance with ASTM Standard E 112. Product PTF was determined using the contact technique previously described and illustrated in FIG. 1. The maximum magnetic permeability of the material perpendicular to the target surface was measured using a LDJ 9600 Vibrating Sample Magnetometer (VSM) in accordance with ASTM Standard A 894-89 (see FIG. 3).

Pure Ni possesses a face-centered-cubic (FCC) crystal structure. The magnetic properties of Ni are crystallographically anisotropic with the [200], [220] and [111] directions being reported to represent the hard, intermediate and easy magnetization directions, respectively. In the Ni system, the intermediate and easy magnetic directions exhibit very similar magnetic characteristics and are noticeably softer than the hard magnetic direction. One means of promoting high PTF is to ensure as high a volume fraction of the easy and intermediate magnetic directions aligned perpendicular to the target surface.

Alignment of easy and intermediate magnetic directions perpendicular to the target surface facilitates magnetic dipole alignment in response to an applied magnetic field and aids in the transmission of the applied field through the bulk of the target material. In order to determine the relative fractions of the different crystallographic directions aligned perpendicular to the target surface, x-ray diffraction (XRD) analysis was conducted. In this analysis, the complete XRD spectra for the final Ni target (derived from ingot #1 using conventional prior art fabrication techniques) was deconvoluted and the % contribution of each of the crystallographic peaks was obtained. FIG. 4 is the XRD spectra of the Ni target and the relative contributions of the different crystallographic directions aligned perpendicular to the target surface are:

Easy magnetic direction [111]: 46%

Intermediate magnetic direction [220]: 16%

Hard magnetic direction [200]: 21%

Other peaks: 17%

The second Ni ingot, #2, was used to develop the new high PTF process of the invention. As in the case of ingot #1, ingot #2 was hot-rolled at about 2000° F. for a total reduction of 40% to heal any as-cast porosity in the ingot. After hot-rolling the ingot was cold water quenched and cold-rolled for a total reduction of 60% and heat-treated at about 1000° F. for 1 hour. Up to this point, the processing of the ingot had two main objectives: (1) to heal any as-cast porosity and (2) to promote a refined recrystallized grain morphology. In addition to high product PTF, a fine grained target morphology is conventionally accepted as improving target sputtering performance. At this stage four coupons were extracted from the plate to determine the optimum warm-rolling practice to utilize. The four coupons were

subjected to the following warm-rolling practices for a total reduction of 65%:

- (1) Clock warm-rolled using between 25% to 50% reductions per pass.
- (2) Cross warm-rolled using between 25% to 50% reductions per pass.
- (3) Cross warm-rolled using between 2% to 25% reductions per pass.
- (4) Straight warm-rolled using between 25% to 50% reductions per pass.

The table below summarizes the PTF and XRD results of the warm-rolling matrix and compares these results to the properties of the target produced from ingot #1 (prior art).

| Process   | % [111] | % [220] | % [200] | R    | PTF (%) |
|-----------|---------|---------|---------|------|---------|
| Prior art | 46      | 16      | 21      | 3.0  | 12      |
| (1)       | 1       | 68      | 17      | 4.1  | 36      |
| (2)       | 16      | 14      | 45      | 0.6  | 35      |
| (3)       | 3       | 47      | 26      | 0.6  | 40      |
| (4)       | 1       | 71      | 7       | 10.3 | 45      |

The parameter R in the table above represents the ratio of the relative percents easy and intermediate magnetic directions divided by the relative percent hard magnetic direction for the different processing routes evaluated. Three main observations can be gleaned from the results in the table above.

First, by comparing the prior art data with that of warm-rolling processes (2) and (3) it can be surmised that even though cross warm-rolling appears to diminish the volume percent of easy and intermediate magnetic direction aligned perpendicular to the target surface, the introduction of internal strain during this process increases the product PTF above that of the prior art.

Second, comparison of the straight warm-rolling process (4) with the different clock- and cross- warm-rolling processes (1), (2) and (3), demonstrates that straight warm-rolling promotes the optimum combination of induced internal strain and crystallographic texture to ensure maximum product PTF. The straight warm-rolling practice appears to be especially effective at minimizing the volume percent of hard magnetic direction aligned perpendicular to the target surface.

Third, comparison of warm-rolling processes (2) and (3) reveals that a lighter pass schedule during rolling is more effective at promoting an increase in product PTF.

These three observations clearly demonstrate the individual contribution of strain and texture in inducing an overall increase in product PTF. Warm-rolling provides the strain component, and the uni-directionality associated with straight warm-rolling provides the textural component. The effect of straight warm-rolling on texture manifests itself in terms of an R parameter greater than about 5. The coupling of these two mechanisms and utilization of a light reduction pass schedule (reduction per pass between 2% to 25% of input plate thickness) yields a product with PTF characteristics higher than conventionally manufactured recrystallized product.

Based on the above analysis, the remaining material from Ingot #2 was straight warm-rolled at temperatures below 1200° F. for a total reduction of 65% using between 2% to 25% reduction per pass. After straight warm-rolling, the plate was machined into a final target product of thickness 0.118" (+/-0.005"). The resulting product exhibited the following microstructural and magnetic properties:

|                                           |                                |
|-------------------------------------------|--------------------------------|
| Grain size =                              | 98 (+/-27) micrometers surface |
|                                           | 86 (+/-32) micrometers center  |
| Grain size gradient (surface-to-center) = | 12 micrometers                 |
| PTF =                                     | 52%                            |
| Umax =                                    | 29                             |

The straight warm-rolled product has a PTF that is more than 4 times greater and a maximum permeability that is more than 7 times lower than the PTF and maximum permeability of the prior art product. Straight warm-rolling promotes a slightly larger grain morphology, but results in a significant reduction in through thickness grain-size gradients.

FIG. 5 represents the grain size distribution of the straight warm-rolled Ni product. Straight warm-rolling can manifest itself in terms of non-equiaxed grains. The grain morphology of the prior art product is essentially equiaxed with an average aspect ratio less than 1.2, whereas the grains in the straight warm-rolled product are slightly elongated with an average aspect ratio of 5.7. FIG. 6 is an XRD spectra of the straight warm-rolled product demonstrating the very strong [220] peak and weak [200] peak compared to the XRD spectra of the prior art product depicted in FIG. 4. The relationship between PTF and Umax is depicted in FIG. 7 and reveals that PTF is inversely exponentially related to Umax. The inverse relationship between PTF and Umax, depicted in FIG. 7 for the case of Ni, generally holds for various alloy compositions such as those described below.

## EXAMPLE 2

### Fabrication of Co Target Product

Three ingots of 99.95 pure Co were vacuum induction melted. Ingot #1 was fabricated using practices available in the prior art: The ingot was hot clock rolled at about 2000° F. for a total reduction of 90%. After hot clock-rolling, the plate was cold water quenched and the plate was machined into a final target product of thickness 0.118" (+/-0.005"). The resulting product exhibited the following microstructural and magnetic properties:

Grain size=12 micrometerssurface  
13 micrometerscenter

Grain size gradient (surface-to-center)=1 micrometers  
PTF=15%

The grains had a fine equiaxed appearance (grain aspect ratio ~1), which arises due to dynamic recrystallization of the Co microstructure during hot-rolling. The average grain sizes at the target surface and center were calculated in accordance with ASTM Standard E 112. Product PTF was determined using the contact technique previously described and illustrated in FIG. 1.

Pure Co, and Co-based alloys, exhibit an allotropic phase transformation response. Thus, depending on the processing route used, pure Co can exhibit an predominantly HCP or combination FCC and HCP crystal structure at ambient temperatures. The magnetic properties of Co are crystallographically anisotropic with the [200], [220] and [111] directions reported as the hard, intermediate and easy magnetization directions, respectively, of the FCC phase and the [100], [101] and [002] reported as the hard, intermediate and easy magnetization directions, respectively, of the HCP phase. FIG. 8 is the XRD spectra of the Co target fabricated from ingot #1, and the relative contributions of the different crystallographic directions aligned perpendicular to the target surface are:

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

928

930

932

934

936

938

940

942

944

946

948

950

952

954

956

958

960

962

964

966

968

970

972

974

976

978

980

982

984

986

988

990

992

994

996

998

1000

1002

1004

1006

1008

1010

1012

1014

1016

1018

1020

1022

1024

1026

1028

1030

1032

1034

1036

1038

1040

1042

1044

1046

1048

1050

1052

1054

1056

1058

1060

1062

1064

1066

1068

1070

1072

1074

1076

1078

1080

1082

1084

1086

1088

1090

1092

1094

1096

1098

1099

1100

1101

1102

1103

1104

1105

1106

1107

1108

1109

1110

1111

1112

1113

1114

1115

1116

1117

1118

1119

1120

1121

1122

## 11

Easy magnetic directions  $[111]_{FCC}$  &  $[002]_{HCP}$  42%  
 Intermediate magnetic directions  $[220]_{FCC}$  &  $[101]_{HCP}$ : 9%  
 Hard magnetic direction  $[200]_{FCC}$  &  $[100]_{HCP}$ : 3% -p1  
 Other peaks: 46%

The table below summarizes the PTF and XRD results of the three different processing routes discussed in the present section.

| Process  | % easy | % intermediate | % hard | R   | PTF (%) |
|----------|--------|----------------|--------|-----|---------|
| Ingot #1 | 15     | 31             | 10     | 4.6 | 15      |
| Ingot #2 | 39     | 6              | 3      | 15  | 50      |
| Ingot #3 | 42     | 9              | 3      | 17  | 70      |

As previously mentioned, the parameter R in the table above represents the ratio of the relative percents easy and intermediate magnetic directions divided by the relative percent hard magnetic direction for the different processing routes evaluated. Examination of this table demonstrates that straight warm-rolling of Co significantly increases alignment of easy and intermediate magnetic directions perpendicular to the target surface at the expense of the hard magnetic direction, and results in a concomitant increase in product PTF. This effect is further obtained by applying a post straight warm-roll anneal to the product. These results are very consistent with the results obtained for the Ni target described in Example 1: straight warm-rolling and a post straight warm-roll annealing promotes the optimum crystallographic texture to ensure maximum product PTF. In the case of pure Co, the effect of straight warm-rolling manifests itself in an R value greater than about 5.

## EXAMPLE 3

## Fabrication of Co—Ni—Cr—Ta Target Product

This example demonstrates that the processing paradigms that apply to pure Co and Ni are equally valid for alloys containing these elements. The underlying result of this example is that the aggressive ferromagnetic properties of Co and Ni dictate the processing route selected. The further addition of supplemental alloying elements does not detract from the fundamental processing paradigms established for pure Co and Ni. Six ingots, three each of the following compositions were cast using vacuum induction melting techniques: Co-10Cr-4Ta and Co-12Cr-4Ta-10Ni.

All the ingots had better than 99.95% purity. All six ingots of Co-10Cr-4Ta and Co-12Cr-4Ta-10Ni were hot-rolled between about 2200° F. for a total reduction of 70%. After hot-rolling, the plates were cold water quenched and heat treated at about 1500° F. for 3 hours and air cooled. At this point each plate of each alloy family saw a distinct processing route:

- (1) After heat treatment, one plate of each alloy was machined into a final target product of thickness 0.350". These plates were processed in accordance with practices available in the prior art.
- (2) Another plate of each alloy was cross warm-rolled at temperatures less than 1200° F. by a total reduction of 20% using a reduction per pass between 2% to 15% of input plate thickness. After cross warm-rolling the plate was cold water quenched and machined into a final target product of thickness 0.350".
- (3) The final plate of each alloy was processed like in (2) except that straight warm-rolling was utilized instead of cross warm-rolling.

## 12

The tables below summarize the microstructural, magnetic and texture properties of the Co-10Cr-4Ta and Co-12Cr-4Ta-10Ni plates fabricated using processing routes (1), (2) and (3).

| Property                                           | Prior art process (1) | Process (2) | Process (3) |
|----------------------------------------------------|-----------------------|-------------|-------------|
| <u>Co—10Cr—4Ta</u>                                 |                       |             |             |
| <u>Microstructure</u>                              |                       |             |             |
| Average grain-size surface                         | 7                     | 55          | 52          |
| Average grain aspect ratio                         | 0.9                   | 1.2         | 1.4         |
| <u>Texture</u>                                     |                       |             |             |
| Easy magnetic direction                            | 6%                    | 6%          | 10%         |
| $[111]_{FCC}$ & $[002]_{HCP}$                      | 35%                   | 36%         | 35%         |
| Inter. magnetic dir. $[220]_{FCC}$ & $[101]_{HCP}$ |                       |             |             |
| Hard magnetic dir.                                 | 9%                    | 6%          | 5%          |
| $[200]_{FCC}$ & $[100]_{HCP}$                      |                       |             |             |
| R                                                  | 4.5                   | 7           | 9           |
| <u>Magnetic</u>                                    |                       |             |             |
| PTF                                                | 27%                   | 39%         | 50%         |
| Umax                                               | 25                    | 22          | 18          |
| <u>Co—12Cr—4Ta—10Ni</u>                            |                       |             |             |
| <u>Microstructure</u>                              |                       |             |             |
| Avg. grain-size surface                            | 25                    | 20          | 25          |
| Avg. grain aspect ratio                            | 1.0                   | 1.3         | 2.4         |
| <u>Texture</u>                                     |                       |             |             |
| Easy magnetic dir.                                 | 22%                   | 22%         | 26%         |
| $[111]_{FCC}$ & $[002]_{HCP}$                      | 28%                   | 25%         | 28%         |
| Inter magnetic dir.                                |                       |             |             |
| $[200]_{FCC}$ & $[101]_{HCP}$                      | 15%                   | 11%         | 8%          |
| Hard magnetic dir.                                 |                       |             |             |
| $[200]_{FCC}$ & $[100]_{HCP}$                      | 3.3                   | 4.3         | 6.8         |
| <u>Magnetic</u>                                    |                       |             |             |
| PTF                                                | 8%                    | 33%         | 47%         |
| Umax                                               | 63                    | 44          | 34          |

An examination of the different grain morphologies arising from processing practices (1), (2) and (3) in Co-10Cr-4Ta and Co-12Cr-4Ta-10Ni, respectively, reveals the larger aspect ratio (2-1.4) of the grains associated with straight warm-rolling. FIGS. 11(a)-(c) and 12(a)-(c) represent the different XRD spectra arising from processing practices (1), (2) and (3) in Co-10Cr-4Ta and Co-12Cr-4Ta-10Ni, respectively. The relative volume % of the different crystallographic peaks was obtained by individually deconvoluting and integrating the areas of the easy, intermediate and hard peaks and dividing by the total integrated area of the spectrum. An approximation to integration for peak area can also be used in which area is defined as peak height times half-width. The XRD spectra in FIGS. 11(a)-(c) and 12(a)-(c) demonstrate that, like pure Co, Co-based alloys are inherently allotropic, their microstructures simultaneously consists of both FCC and HCP phases. FIGS. 13(a)-(c) and 14(a)-(c) represent the VSM data used for calculating maximum permeability for Co-10Cr-4Ta and Co-12Cr-4Ta-10Ni processed using routes (1), (2) and (3), respectively.

In the following discussion, the data for Co-10Cr-4Ta and Co-12Cr-4Ta-10Ni will be placed in context with the data

for Ni and Co to illustrate the general interrelationship between the processing techniques, microstructural properties and magnetic properties disclosed in the present invention. FIGS. 15, 16, and 17 compare the effect of prior art processing, cross or clock warm-roll processing and straight warm-roll processing on product PTF, texture (represented by the previously defined parameter R) and grain aspect ratio for all the materials discussed thus far. Note, in these figures X-WR refers to cross, clock or multi-axial warm-rolling and SWR refers to straight or uniaxial warm-rolling.

FIG. 15 demonstrates that warm-rolling promotes a general increase in product PTF compared to product fabricated without the warm-rolling process. Irrespective of the directionality of warm-rolling, the utilization of this process will result in a product PTF in excess of 30% if conducted according to the principles outlined in this invention. Ensuring uniaxial or straight warm-rolling promotes a further increase in product PTF over and above cross or clock rolling, and for all the alloys claimed will result in product PTF greater than 45% if conducted according to the principles outlined in this invention. FIG. 15 illustrates that warm-rolling alone is not sufficient to maximize product PTF, the constraint of straight or uniaxial warm-rolling is integral to product PTF maximization.

FIG. 16 demonstrates why straight warm-rolling results in maximization of product PTF. As previously discussed, it is hypothesized that warm-rolling increases product PTF by inducing internal strain (which is known to reduce inherent material permeability) and increasing the alignment of easy and intermediate magnetic directions aligned perpendicular to the target surface at the expense of hard magnetic directions aligned perpendicular to the target surface (the parameter R quantifies the relative contribution of easy and intermediate magnetic directions aligned perpendicular to the target surface divided by the contribution of hard magnetic directions aligned perpendicular to the target surface).

FIG. 16 also demonstrates that multi-axial warm-rolling most likely promotes an increase in PTF predominantly by virtue of increasing the internal strain in the material, and in some cases by promoting an increase in the contribution of easy and intermediate magnetic crystallographic directions aligned perpendicular to the target surface. For some materials multi-axial warm-rolling increases the value of R and in other materials it decreases the value of R suggesting that its effect of increasing PTF via texture manipulation is inconsistent and un-optimized. In contrast, uniaxial warm-rolling overwhelmingly increases R compared to multi-axial warm-rolling and prior art fabrication techniques.

Uniaxial warm-rolling appears to be particularly effective at increasing R by strongly reducing the contribution of hard magnetic directions aligned perpendicular to the target surface. FIG. 21 shows that PTF maximization by uniaxial warm-rolling occurs by: one, introduction of internal strain into the product microstructure and two, by maximizing the contribution of easy and intermediate magnetic crystallographic directions aligned perpendicular to the target surface at the explicit expense of the hard magnetic crystallographic directions. FIG. 21 further demonstrates that application of uniaxial warm-rolling to the product claimed in the present invention will promote an R value greater than 5.

FIG. 17 demonstrates that application of uniaxial warm-rolling without a post warm-roll anneal or heat treatment promotes an elongated grain morphology with an average aspect ratio greater than 1.4 for the alloys claimed in the present invention. The grain elongation is a microstructural manifestation of the uni-directional macroscopic deformation.

FIG. 18 is an expanded representation of FIG. 7 and demonstrates the inverse exponential relationship between PTF and maximum magnetic permeability. For the alloys claimed in the present investigation, increasing product PTF appears to be directly correlated to decreasing the maximum magnetic permeability of the product.

In summary, FIGS. 15 to 18 show that uniaxial straight warm-rolling will increase product PTF to values greater than 45% which correlates to maximum material permeabilities less than 37, and can be directly related to texture constant R values greater than 5 and microstructural grain width-to-length aspect ratios greater than 1.4.

#### EXAMPLE 4

##### Fabrication of Co—Cr—(Pt.Ta.B) Target Product

The purpose of this example is to further demonstrate the transcendence of the positive impact of uniaxial warm-rolling on PTF and alloy chemistry. Two ingots each of the following alloys were fabricated for experimentation: Co-16Cr-11Pt, Co-15Cr-6Pt-4Ta and Co-20Cr-10Pt-6B. All the ingots had better than 99.95% purity. Similar to Example 3, all the ingots were hot-rolled at about 2200° F. for a total reduction of 70%. After hot-rolling, the plates were cold water quenched and heat treated at about 1500° F. for about 3 hours and air cooled. At this point, one plate from each alloy was machined into a final target product of thickness 0.350". These plates were processed in accordance with practices available in the prior art. The second plate of each alloy uniaxially warm-rolled at temperatures less than 1200° F. by a total reduction of 10% using a reduction per pass between 2% to 5% of input plate thickness. After uniaxial warm-rolling, the plate was cold water quenched and machined into a final target product of thickness 0.350".

The table below compares the PTF for each of the alloys fabricated using prior art practices and the new uniaxial warm-roll practice.

| Alloy           | PTF<br>(prior art practice) | PTF<br>(uniaxial warm-roll<br>practice) |
|-----------------|-----------------------------|-----------------------------------------|
| Co-16Cr-11Pt    | 10%                         | 68%                                     |
| Co-15Cr-6Pt-4Ta | 35%                         | 64%                                     |
| Co-20Cr-10Pt-6B | 27%                         | 60%                                     |

The significant impact of uniaxial warm-rolling on product PTF is very evident from this example. As previously discussed, utilization of warm-rolling, uniaxial warm-rolling in particular, during the fabrication of magnetic data storage targets results in a product that yields maximum material utilization and result in optimum deposited film thickness uniformity.

What is claimed is:

1. A method for forming a magnetic sheet material having improved Pass Through Flux comprising the steps of:

(a) casting a magnetic metal or metal alloy, said magnetic metal or metal alloy being selected from the group consisting of those of the formula:



wherein a-d are atomic weight % basis and wherein a is 0-100%, b is 0-40%, c is 0-8%, and d is the remainder, and wherein the magnetic metal or metal alloy may contain from 0- 30% (atomic), based on

**15**

- 100% of the metal or alloy, of one or more secondary elements selected from the group consisting of Pt, B, Si, Zr, Fe, W, Mo, V, Nb, Hf, Ti, and Sm;
- (b) hot-rolling the metal or metal alloy, thereby forming a sheet
- (c) cold water quenching the sheet formed in step (b); and
- (d) warm-rolling the quenched sheet of step (c) at a temperature of less than about 1400° F. to achieve a reduction in sheet thickness of at least about 15%, thereby forming a magnetic sheet material.
2. A method according to claim 1, wherein the improved Pass Through Flux for the magnetic sheet material is at least about 30%.
3. A method according to claim 2, wherein the Pass Through Flux is between about 40% and 95%.
4. A method according to claim 1, wherein said magnetic sheet material has an average grain length-to-width aspect ratio of greater than about 1:1 in the rolling direction.
5. A method according to claim 1, wherein said warm rolling step is conducted at temperatures of less than 1200° F.
6. A method according to claim 1, wherein said warm rolling step is conducted in multiple passes.
7. A method according to claim 1, wherein said warm rolling step is conducted by uniaxially warm rolling.
8. A method as claimed in claim 1, wherein the reduction in sheet thickness during said warm-rolling step is about 15% to about 75%.
9. A method as claimed in claim 1, wherein the reduction in sheet thickness during said warm-rolling step is at least about 50%.
10. A method as claimed in claim 1, wherein the reduction in sheet thickness during said warm-rolling step is at least about 85%.
11. A method as claimed in claim 10, further including the step of post annealing the warm rolled sheet of step (d).

**16**

12. A method as claimed in claim 11, further including pre-annealing the sheet material prior to step (d).
13. A method as claimed in claim 1, wherein the warm-rolling step (d) comprises warm-rolling at a temperature of about 600° to 1100° F.
14. A method as claimed in claim 1, wherein the warm-rolling of step (d) comprises warm-rolling the sheet in a clockwise or counterclockwise direction.
15. A method as claimed in claim 1, wherein the warm-rolling of step (d) comprises warm-rolling by rolling the sheet alternatively at 90° angles from a previous rolling step.
16. A method as claimed in claim 1, wherein the warm-rolling of step (d) comprises warm-rolling the sheet in the same direction for all rolling steps.
17. A method as claimed in claim 16, wherein the reduction in sheet thickness during the warm-rolling step (d) is at least about 30%.
18. A method as claimed in claim 17, wherein the warm-rolling is performed in at least two passes and wherein the sheet thickness reduction per pass is from about 2 to about 25%.
19. A method as claimed in claim 18, further including the step of (e) post annealing the warm-rolled sheet material of step (d).
20. A method as claimed in claim 19, further including pre-annealing the sheet material prior to step (d).
21. In a method for forming a magnetic sheet material from cobalt or a cobalt alloy, the improvement comprising warm-rolling a cobalt or cobalt alloy sheet material at a temperature of less than about 1400° F. to achieve a reduction in sheet thickness of at least about 15%, and wherein said warm-rolling is effective to provide a Pass Through Flux for the sheet material of 40% to 95%.

\* \* \* \* \*